

July 1, 1958

F. D. ROSI

2,841,559

METHOD OF DOPING SEMI-CONDUCTIVE MATERIALS

Filed April 27, 1955



FIG. 1



FIG. 2

INVENTOR.  
FRED D. ROSI  
BY  
S. L. Whittaker  
ATTORNEY

2,841,559

## METHOD OF DOPING SEMI-CONDUCTIVE MATERIALS

Fred D. Rosi, Plainsboro, N. J., assignor to Radio Corporation of America, a corporation of Delaware

Application April 27, 1955, Serial No. 504,189

10 Claims. (Cl. 252—62.3)

This invention relates generally to an improved method for alloying a relatively low boiling or sublimation point material with a relatively high melting point semi-conductive material. More particularly, but not necessarily exclusively, the invention relates to the alloying of low boiling or low sublimation point conductivity-type-determining impurities with high melting point molten semi-conductive materials such as germanium and silicon.

It is known to control the type of conductivity of semi-conductive materials by introducing thereinto small amounts of certain foreign materials generally termed "impurities." The introduction of such impurities into semi-conductive materials is usually referred to as "doping." The type of conductivity established in the semi-conductor is dependent upon the electron configuration of the atoms of the impurity material and of the host crystal. Thus, a substance whose atoms are capable of giving up electrons to the atoms of a particular substance is termed a "donor" impurity, and since there is a surplus of electrons available to carry a current, the semi-conductor so doped is deemed to be of n-type (negative) conductivity. On the other hand, a substance whose atoms are capable of borrowing or accepting electrons is termed an "acceptor" impurity, and since there is a shortage of electrons in the crystal lattice available for current conduction, the semi-conductor so doped is deemed to be of p-type (positive) conductivity.

The usual and most directly convenient manner of introducing impurities into a semi-conductor is to add the impurity into a melt of the semi-conductive material. Some semi-conductive materials have relatively high melting points. Silicon, for example, melts at 1420° C. Great difficulty is therefore encountered in attempting to dope such high melting point semi-conductors with lower boiling point impurities inasmuch as such impurities boil-off either prior to introduction into the semi-conductor melt or before alloying with the molten semi-conductor. This is especially true when the boiling point of the impurity is greatly lower than the semi-conductor melting point. Some impurities sublime rather than boil at relatively low temperatures and it is intended throughout the instant application to include—sublimation temperature—in the phrase "boiling point". Typical impurities having boiling points sufficiently low to cause difficulty in doping high melting point semi-conductors therewith are antimony (boiling point 1380° C.), red phosphorus (boiling point 280° C.), arsenic (sublimation point 615° C.), tellurium (boiling point 1390° C.), selenium (boiling point 688° C.), lithium (boiling point 1336° C.), cesium (boiling point 670° C.), calcium (boiling point 1240° C.), and magnesium (boiling point 1107° C.). The same is also true for the semi-conductor germanium which melts at 940° C.

It is therefore an object of this invention to provide an improved method of alloying an impurity material with a semi-conductive material having a melting point either

about the same or higher than the boiling point of said impurity material.

Another object of this invention is to provide an improved method of doping a growing crystal of a semi-conductive material such as germanium or silicon with an impurity having a boiling point lower than the melting points of said semi-conductive materials without boiling-off the impurity.

These and other objects and advantages are accomplished according to the invention by employing a relatively high boiling point compound one of the constituents of which is the relatively volatile impurity material with which it is desired to dope a melt of a semi-conductive material such as germanium or silicon. The other constituent of the compound is an element whose valence is the same as that of the semi-conductive material. Due to its equivalency such an element will not ionize in the semi-conductive material and affect its conductivity. An example of such a compound for germanium or silicon is lead selenide. This compound is either added as a solid or melted and then added to the molten semi-conductive material. The molten semi-conductive material is then re-frozen as either a single crystal or polycrystalline ingot. Since the boiling point of the compound is much higher than the boiling point of the impurity material uncombined and is also higher than the melting point of the semi-conductive material, the relatively low boiling point impurity can be introduced into the molten semi-conductive material as a constituent of a compound which will not boil-off and become lost.

The invention will be described in greater detail by reference to the accompanying drawing wherein:

Figure 1 is a cross-sectional, elevational view of an elongated crucible being drawn through an induction type furnace; and

Figure 2 is a partially cross-sectional, elevational view of an apparatus for pulling a crystal from a melt.

Referring to the drawing, a semi-conductive material such as silicon can be doped with a volatile impurity such as selenium employing the apparatus shown in Figure 1. An elongated boatlike crucible 6 of graphite is charged with a rod-shaped piece of base material 2 such as silicon. If it is desired to produce a single crystal of silicon, then a seed crystal 4 of silicon is placed at one end 40 of the crucible 6 close to but not in contact with the silicon charge. Between the seed crystal 4 and the silicon charge 2 a stoichiometric compound 7 of selenium and lead is placed. The lead selenide may be in any convenient form, such as pellets, for example. To produce a polycrystalline ingot of silicon the seed crystal 4 is omitted.

The crucible is placed within a quartz tubular enclosure 11 and is gradually drawn at about 2.5 inches per hour or less, for example, through a ring-shaped induction heating element 12 starting at the seed crystal end of the crucible. The crucible is supported within the enclosure 11 by a ring-shaped member 5. At the start of the pulling operation, when the temperature reaches the melting point of the silicon, part of the seed 4 melts as well as all of the lead-selenide alloy 7, and the adjacent part of the silicon charge 2. As the crucible with its contents is drawn through the heating element 12, successive segments of the charge 2 are melted. The molten lead selenide dissociates in the molten silicon thus providing a quantity of selenium atoms in the silicon melt.

By reason of the segregation coefficient of selenium in silicon, which is defined as the ratio of the impurity (selenium) concentration in the solid side of the interface of a growing crystal to the concentration on the liquid side of the interface, some of the selenium atoms available in the melt will segregate to and freeze-out with

the silicon. The segregation coefficient of selenium in silicon is not known. However, it is known that segregation of some of the selenium atoms in a silicon melt does occur and are thus able to establish the crystal conductivity-type as the molten materials re-crystallize as an extension of the seed crystal lattice. Re-crystallization occurs as the crucible leaves the heat zone created by the heating element 12. Since the melting point of the compound lead selenide is 1088° C., it will have a much higher boiling point, and, while this boiling point is not known precisely, it is higher than the melting point of the silicon. Therefore, none of the selenium in the compound will be lost by vaporization and is available to contribute to the conductivity of the silicon single crystal being grown.

With such a compound, the conductivity of the silicon is affected only by the selenium atoms entering the single crystal lattice of silicon since the lead, being tetravalent, and having no free electrons or holes, does not ionize in the silicon lattice.

In one example, 40 grams of p-type silicon of 50 ohm-cm. resistivity doped with 0.94 gram of lead selenide results in a single crystal of silicon having a resistivity of 1.5-2.5 ohm-cm. The conductivity of the single crystal produced from this charge is n-type.

In another example, semi-conductive silicon is doped with a relatively low boiling point impurity such as cesium employing the apparatus shown in Figure 2. It should be understood, however, that the apparatus shown in Figure 1 could likewise be employed, if desired, in the instant example. In Figure 2, a pot-type crucible 18 which may be of silica, for example, is supported by a pedestal 9 of fire-brick or other heat-insulating material in a quartz container 7, and heated by conventional means (not shown). The crucible is charged with silicon 20, for example 50 grams, and a seed of single crystal silicon 23 attached to a withdrawing apparatus 24 is touched onto the surface of the molten silicon in the crucible. As the seed 23 is slowly withdrawn, an elongated single crystal 22 is attached thereto. The seed crystal is withdrawn, at a rate of 0.5 cm. per hour or less, for example. A stoichiometric compound of cesium stannide ( $Cs_2Sn$ ) is added to the silicon melt in either pellet or powder form where it melts and dissociates throughout the molten mass. Again, by reason of the segregation coefficient of cesium in silicon, some of the cesium atoms in the melt segregate to and freeze-out as an extension of the seed crystal lattice and thus contribute to the conductivity of the silicon single crystal being grown. Since the cesium stannide has a melting point (1400° C.) which is about the same as that of silicon, its boiling point will be still higher. Therefore, none of the cesium carried in the compound will be lost by vaporization and is available to establish the conductivity of the silicon single crystal being grown.

With a compound of cesium and tin, the conductivity of the silicon is affected only by the cesium atoms entering the single crystal lattice of silicon. The tin, being tetravalent, does not ionize in the silicon lattice and contribute conduction electrons or holes.

When doping tetravalent semi-conductors according to the invention, a binary compound of the doping element and an element which is tetravalent is selected. As has been indicated, the reason for choosing a tetravalent element is to insure that the conductivity of the grown crystal will be determined only by the impurity element itself. That is, since the compound dissociates in the molten semi-conductor, the conductivity of the crystal might be affected by both constituents of the compound if one were not tetravalent.

The following binary compounds may be employed to dope tetravalent semi-conductors such as silicon and germanium. For doping with selenium, PbSe has the requisite melting and boiling point (melting at 1088° C.). For doping with tellurium, SnTe (melting at 917°

75 C.) may be employed; and for doping with magnesium,  $Mg_2Sn$  (melting at 778° C.). Cesium may be introduced by the compound  $Cs_2Sn$  (melting at 1400° C.). Lithium may be introduced by the compounds  $Li_7Sn$  (melting at 783° C.) or  $Li_7Pb_2$  (melting at 726°C.). Calcium likewise may be introduced by the following compounds:  $CaSi$  (melting at 1245° C.),  $Ca_2Pb$  (melting at 1110° C.), and  $CaTi_2$  (melting at 1450° C.).

It is to be noted that only melting points of the enumerated compounds have been given. This is because the precise boiling points are not known. It is, however, certain that the boiling points of these compounds will be sufficiently higher than their melting points so that the compounds may be introduced in the various molten semi-conductors without their boiling off.

What is claimed is:

1. The method of alloying a conductivity-type-determining material with a semi-conductive element selected from the class consisting of germanium and silicon and having a particular valence, the melting point of said semi-conductive element being higher than the boiling point of said conductivity-type-determining material, comprising the step of: adding into a melt of said semi-conductive element a compound consisting of said conductivity-

20 type-determining material and an element having a valence the same as that of said semi-conductive element, the boiling point of said compound being higher than the melting point of said semi-conductive element.

2. The method of alloying a conductivity-type-determining impurity material selected from the class consisting of selenium, magnesium, lithium, cesium, calcium, and tellurium with a semi-conductive material selected from the class consisting of germanium and silicon, the melting point of said semi-conductive material being higher than the boiling point of said impurity material, comprising the step of: adding into a melt of said semi-conductive material a binary compound of a tetravalent element and said impurity material, the boiling point of said compound being higher than the melting point of said semi-conductive material.

3. The method of alloying a conductivity-type-determining impurity material with a semi-conductive material selected from the class consisting of germanium and silicon, the melting point of said semi-conductive material being higher than the boiling point of said impurity material, comprising the step of: adding into a melt of said semi-conductive material a compound selected from the class consisting of:  $PbSe$ ,  $Mg_2Sn$ ,  $Li_7Pb_2$ ,  $Li_7Sn$ ,  $Cs_2Sn$ ,  $CaSi$ ,  $Ca_2Pb$ ,  $SnTe$ ,  $PbTe$ , and  $CaTi_2$ .

4. The method of growing a single crystal of a semi-conductive element selected from the class consisting of germanium and silicon and having a particular valence and containing a conductivity-type-determining impurity material whose boiling point is lower than the melting point of said semi-conductive element comprising the steps of: preparing a melt of said semi-conductive element and a compound consisting essentially of said impurity material and an element having a valence the same as that of said semi-conductive element, said compound having a boiling point higher than the melting point of said semi-conductive element, and initiating and maintaining single crystalline growth of said semi-conductive element from said melt.

5. The method of growing a single crystal of a semi-conductive element selected from the class consisting of germanium and silicon and having a particular valence and containing a conductivity-type-determining impurity material whose boiling point is lower than the melting point of said semi-conductive element comprising the steps of: preparing a melt of said semi-conductive element and a compound consisting essentially of said impurity material and an element having a valence the same as that of said semi-conductive element, said compound having a boiling point higher than the melting point of said semi-conductive element, contacting a seed crystal

of said semi-conductive element to said melt until a single crystal of said semi-conductive element starts to grow attached thereto, and relatively moving said seed crystal away from said melt as said single crystal continues to grow.

6. The method of growing a single crystal of semi-conductive element selected from the class consisting of germanium and silicon and having a particular valence and containing a conductivity-type-determining impurity material whose boiling point is lower than the melting point of said semi-conductive element by horizontally zone-melting an elongated body of said semi-conductive element comprising the steps of: placing a mass of a compound consisting essentially of said impurity material and an element having a valence the same as that of said semi-conductive element at one end of said elongated body of said semi-conductive element, said compound having a boiling point higher than the melting point of said semi-conductive element, melting said compound mass and a portion of said end of said elongated body of semi-conductive element, initiating single crystalline growth of said semi-conductive element from said melt, and thereafter melting and freezing-out successive adjacent portions of said elongated body of said semi-conductive element whereby a single crystal of said semi-conductive element is grown containing said impurity material.

7. The method according to claim 6 wherein said single crystalline growth is initiated by contacting a seed crystal of said semi-conductive element to said melt.

8. The method of growing a single crystal of silicon containing impurity centers of selenium comprising the steps of: preparing a melt of silicon and lead selenide, and initiating and maintaining single crystalline growth of said silicon from said melt.

9. The method according to claim 8 wherein said single crystalline growth is initiated by contacting a seed crystal of silicon to said melt, and thereafter maintaining said single crystalline growth by relatively moving said seed crystal away from said melt.

10. The method according to claim 9 wherein said melt is prepared by melting an end portion of an elongated body of said silicon together with a mass of said lead selenide, and said single crystal is grown by horizontally zone-melting successive adjacent portions of said elongated body of said silicon.

References Cited in the file of this patent

UNITED STATES PATENTS

2,530,110 Woodyard ----- Nov. 14, 1950